

Jan. 21, 1936.

J. E. PERRY ET AL

2,028,244

STEEL INGOT

Original Filed July 5, 1923 2 Sheets-Sheet 1



Fig. 1.

Fig. 2.



Fig. 3.

INVENTORS  
John E. Perry  
and William Haig Ramage  
George Ramage  
ATTORNEY

Jan. 21, 1936.

J. E. PERRY ET AL

2,028,244

STEEL INGOT

Original Filed July 5, 1923 2 Sheets-Sheet 2



By

INVENTORS  
John E. Perry  
and William Haig Ramage  
George Ramsey  
their ATTORNEY

## UNITED STATES PATENT OFFICE

2,028,244

## STEEL INGOT

John E. Perry, Youngstown, and William Haig Ramage, Girard, Ohio, assignors to Valley Mould and Iron Corporation, Hubbard, Ohio, a corporation of New York

Original application July 5, 1928, Serial No. 290,329. Divided and this application August 26, 1929, Serial No. 388,293. In Canada July 24, 1928

9 Claims. (Cl. 22—218)

The present invention relates broadly to the metallurgy of steel and more especially to a steel ingot. The present application comprises a division of our application Serial No. 290,329, filed

5 July 5, 1928.

The present invention relates to an ingot of steel having corrugated surfaces of a novel characteristic and wherein the surface cracks and defects adjacent the surface of the ingot are eliminated and where the corrugations in the ingot are arranged particularly with reference to facilitating rolling of the ingot.

Ingots of the prior art having relatively high salients of small cross section formed on small radii not only tend to trap segregates when the ingot is frozen, but also have weakness caused by entangled columnar crystals in the salients. These high salients tend to decarburize or burn on the tops when being reheated in the soaking pit for rolling or working. This results in weakened longitudinal planes extending into the ingot from the top of the salients and articles fabricated from such ingots show faults over these weakened areas in the finished product, which areas correspond to the crests of the small salients.

The present invention comprises an ingot wherein the curvature of the salients and of the valleys between the salients are such that when the ingot is being cast, columnar crystals in the ingot which grow at right angles to the surface of the mold do not tend to focus within the zone of direct chill in the ingot produced from the cold walls of the mold. The axes of the radii upon which the salients and the valleys or non-salient portions of the surface of the ingot are formed are such that the columnar crystals in the ingot, if extended, do come to a focus within the zones of axial crystals and the inner ends of the columnar crystals do not overlap or intersect with each other. Therefore, the ingot does not contain concentrates which are trapped by the ends of the columnar crystals as would be the case if these crystals did actually intersect and focus within their own zones.

From a crystalline standpoint, the radii of the non-salient portions of the surface of the ingot is not so important as the radii of the salient portions, but in practice, it has been found that the valleys or non-salient portions should be such as to avoid surface defects, which may occur in working the ingot when the valleys are on very small radii and also to prevent the free growth of columnar crystals without bringing the inner ends of these crystals into interlacing contact

with each other. The inner ends of these columnar crystals comprise a wavy zone surrounding and securely locked to the zone of axial crystals in the center portion of the ingot.

Another important feature of the invention resides in the arrangement of the salients on the ingots in that the initial roll contacting tops of the salients are parallel to each other and to center planes at right angles to the mid sections of the ingot surface. This results in the salients running in a straight line under the rolls of a rolling mill and thus prevents any cross or diagonal rolling on the surface of the ingot. The dimensions of the salients on the surface of the ingot are formed throughout the length of the ingot, and this also obviates rolling strains on the salients and permits uniform heating of the salients when the ingot is in the soaking pit. Where the surfaces of the ingot are tapered as may be the case in rectangular ingots, the maintaining of the salients and valleys throughout the length of the ingot may be accomplished by providing small flat narrow rectangular areas on the sides of the ingots adjacent the corners and which areas are located between the corner curved surfaces of the adjacent salients on the ingot.

Increased height of salients on the ingot gives increased strength to the ingot skin. In rolling practice, however, there is a maximum height which is allowable for any given cross sectional sizes of ingot. However, the size of the ingot determines the number of proper salients which may be placed in a side thereof. Using this proper number of salients with the form of curvature such as will result in correct crystallization in the ingot, the maximum height of the salient is obtained by having the areas of the valleys between the salients relatively small.

Other and further objects of the present invention will in part be obvious and will in part be pointed out hereinafter by reference to the accompanying drawings, forming a part of this specification.

Realizing that the present invention may be embodied in structures other than those specifically disclosed, it is to be understood that the disclosure herewith is illustrative and not in the limiting sense.

Fig. 1 is a longitudinal view of the exterior of one side of a rectangular ingot in accordance with the present invention.

Fig. 2 is a view similar to Fig. 1 and showing a portion of the ingot broken away to clearly illustrate the relation between the columnar and axial crystals.

Fig. 3 is a cross sectional plan view taken on line 3-3 of Fig. 1.

Fig. 4 illustrates a detail portion comprising a section adjacent one side of an ingot in accordance with the present invention and with the salients joined by long non-salient portions.

Fig. 5 is a view similar to Fig. 4 showing these salients joined by short non-salient portions.

Fig. 6 is a view similar to Figs. 4 and 5 and 10 wherein the salients are of small radii but low depth.

Referring now to the drawings and more especially to Figs. 1, 2, and 3, which illustrate an ingot in accordance with the present invention, 15 which is provided with salients 1, in the present case comprising two salients (which number may be increased as desired) between each corner surface 2, and joined at the mid-section of the side wall of the ingot by a non-salient or valley 4. 20 The salients 1 have their top-most portions extending parallel throughout the length of the ingot, as indicated by lines 5 and 6 of Fig. 1. The ingots may be tapered slightly with the bottom width of the side being slightly greater 25 than the top width thereof, and flat surfaces 7 and 8 (shown in Fig. 1 in dotted lines in exaggeration) occur between the corner surfaces 2 and the adjacent salient ribs 1. These surfaces 7 and 8 are referred to as "flat" but it is to be understood that the term "flat" is merely relative. 30 These surfaces may be somewhat curved, and the feature which is emphasized is that the salient ribs 1 are made with their initial roll contacting top portions parallel without distortion of the 35 corner surfaces, and with the salient ribs 1 being substantially the same width and height throughout the length of the ingot. An extremely important feature of the present ingot is that the ribs 1 and the valleys 4 are formed upon such curvature (when considered in cross section) 40 that the growth of columnar crystals, when the ingot is freezing, is such as not to focus within the zone of chill produced by the chill mold wall in which the ingot is cast. In the preferred embodiment of the invention the axes 9 of the radii 45 10 on which the salient ribs are formed are in the zone A of axial crystals of the ingot, and within the zone B of the normal effect of chill of the mold on the crystallization of the steel of the ingot. An ingot in accordance with this construction has a crystalline structure wherein the columnar crystals occur at substantially right angles to the surface of the ingot, but do not come to focus within the zone B and, therefore, the ingot is free from inclusions which otherwise 55 would occur at about this zone.

A further advantage of an ingot in accordance with the present invention is that the zone represented by the dotted line C, Figs. 2 and 3, where the columnar crystals meet the axial crystals, is such that these two types of crystals interlock with each other in such manner as to thoroughly tie the two types of crystals together. It is to be understood that while this interlocking zone between the columnar crystals and the axial crystals 60 is indicated by dotted line C, the zone is of substantial width so that this dotted line indicates the general location of the zone rather than the absolute definite limits of the zone. The radii 11 of the corners are preferably of such length that the axes 12 of these corner radii are also well within the zone A of axial crystallization, and the corners 2 are preferably rounded on uniform radii for the full length of the ingot.

Fig. 4 is a detailed sectional portion of the side

of an ingot taken at right angles to the salient ribs and shows the salients 14 and 15, which are on radii of the same length, being joined by a relatively long radius non-salient portion 16, which is tangent at its extremities to the curves of the salients 14 and 15. The axes 17 of the radii 18 are located well within the zone of axial crystals A. In this construction the general tend of the growth of columnar crystals is in accordance with the lines 19 and it will be observed that these lines do not focus within the zone B, representing the normal depth of the chill in the ingot due to the effect of the mold in which the ingot is cast.

Fig. 5 is a view similar to Fig. 4 with the salients 20 and 21 formed upon the same radii as the salients shown in Fig. 4, but with the non-salient portion 22 on a much shorter radius than the non-salient portion 16 of Fig. 4. In the type of ingot shown in Fig. 5 a much deeper salient is provided in that the tangents on each side of the non-salient portion where this portion joins the salients are closer together than in the construction shown in Fig. 4. In other words, the side wall length of the salients is extended further than the side wall of the salients in Fig. 4. This produces a stiffer ingot during the time the ingot is freezing and also produces a somewhat longer surface skin on the side of the ingot. The lines 24 illustrate the general direction of the columnar crystals under the construction shown in Fig. 5 and while more crystals are directed toward the axes on which the salients are formed, none of these lines 24 come to a focus within the zone B representing the mold wall chill and consequently there is no tendency of trapping inclusions in the zone between the axial and the columnar crystals.

Fig. 6 illustrates small salients 25 upon radii 26 formed on axes 27 and also small non-salient portions 28. This produces the side wall on the ingot in which the height of the salients is relatively low. It will be observed that the axes 27 for the salients are located very close to the edge of the chill zone B. While, as above specified, columnar crystals tend to grow at substantially right angles to the ingot side wall, the actual growth of these crystals or location of these crystals in the ingot is influenced by the surface on the ingot, as for example, in Fig. 6, the columnar crystals 29 from the salients 25 are influenced by the relation of the columnar crystals from the non-salients 28. Under these conditions the columnar crystals 30 beneath the non-salients 28 spread out fanwise with plenty of space to grow in and therefore relieve the concentration pressure on the inner ends of the columnar crystals 29. In this way practically none of the crystals directly under the salients tends to focus within the zone chill but on the other hand tends to focus, as expanded, between the point 31 and the axis 27 on which the small salients are formed. This condition obviates the formation of any cleavage plane by the focusing of the columnar crystals and consequently the crystallization in the ingot is not detrimental to the ingot. On the other hand, an ingot surface is provided which may stretch under rolling without breaking and furthermore, the small salients support the ingot during the freezing thereof.

The present invention produces ingots not only having improved skin surfaces, but which are also better ingots from a metallurgical standpoint in that the curvatures of the salients on the surface of the ingots are such as to permit

proper freezing and crystallization of the steel without the trapping of harmful inclusions at the juncture between the columnar crystals and the axial crystals. Furthermore, since the tops of the salients are parallel throughout the length of the 5 ingot, there is no cross rolling when the ingot passes through the rolling mill.

What we claim is:—

1. An article of manufacture comprising an 10 ingot of steel tapering from one end toward the other and having salient portions on the longitudinal surfaces thereof, said salient portions on each side being parallel to salient portions on the same side and extending the full length of 15 said ingot, said salient portions being remote from the corners of said ingot.

2. An article of manufacture comprising an 20 ingot of steel tapering from one end toward the other and having salient portions extending the full length of said ingot, said salient portions being of the same width throughout the length of the ingot, said salient portions being remote from the corners of the ingot.

3. An article of manufacture comprising an 25 ingot of steel tapering from one end toward the other and having salient portions on the surfaces thereof, the depth of said salient portions being uniform throughout their length.

4. An article of manufacture comprising an 30 ingot of steel of rectangular cross section and tapering from one end toward the other and having salient portions on the surfaces thereof, the depth of said salient portions on a side being uniform throughout their length.

35 5. As an article of manufacture, an ingot of steel having longitudinal taper and with salient portions on the sides of said ingot, the salient portions on each side being parallel to other

salient portions on the same side, the corners of said ingot being rounded on a uniform radius throughout the length of the ingot, and with narrow triangular areas extending lengthwise of the ingot adjacent to said corners. 5

6. As an article of manufacture, an ingot of steel tapering from one end toward the other and with salient portions on the sides of said ingot, the salient portions on each side being parallel to other salient portions on the same side, the corners of said ingot being rounded throughout the length of the ingot, the salient portions and said corners comprising surfaces generated on radii of a length greater than the depth of the 10 columnar crystalline zone of the ingot. 15

7. As an article of manufacture, a steel ingot tapering from one end toward the other and having salients on the sides thereof, said salients being formed upon radii having axes extending parallel to the surface of the ingot and parallel 20 to each other axis on the same side of the ingot, and non-salients formed on radii of a lesser length than the radii of the salients.

8. As an article of manufacture, an ingot of steel having longitudinally tapered sides and with 25 salient portions on the sides thereof, said salient portions being formed on radii of uniform length and having axes extending parallel to the surface of the ingot and with said axes being located in the zone of axial crystals of the ingot. 30

9. A longitudinally tapered metallic ingot having a substantially rectangular cross section with rounded corners and salients superimposed on the sides of said ingot comprising segments of cylinders extending lengthwise of said ingot. 35

JOHN E. PERRY.

WILLIAM HAIG RAMAGE.